

## UNITED STATES PATENT OFFICE

2,285,028

## ROSIN SIZE EMULSION

Edmund A. Georgi and Arthur L. Osterhof, Wilmington, Del., assignors to Hercules Powder Company, Wilmington, Del., a corporation of Delaware

No Drawing. Application September 16, 1940,  
Serial No. 357,007

4 Claims. (Cl. 106—238)

This invention concerns dilute rosin size emulsions and in particular relates to substantially non-foaming and non-sludging aqueous emulsions of saponified rosin adapted to use in paper-sizing.

At the present time, the sizing of paper is usually effected by adding to the paper stock prior to the formation of the paper web on the paper-making machine, a dilute aqueous emulsion of completely or partially saponified rosin from which a complex resinate is subsequently precipitated on the stock fibres by means of alum or other suitable precipitant. Such saponified rosin size emulsions are in general prepared by reacting gum or wood rosin with an alkali, such as sodium hydroxide or sodium carbonate, whereby at least a part of the abietic and other rosin acids present in the rosin are converted into their water-soluble alkali-metal salts, and thereafter forming a dilute emulsion of the reaction product in water. Emulsification is readily effected since the alkali-metal resinates act as emulsifying agents for the unsaponified portion of the rosin.

Although rosin size emulsions prepared in this manner are widely used in the paper-sizing art, they possess several serious disadvantages, among which is a tendency to induce frothing or foaming of the sized stock during the subsequent paper-forming operations. Foam not only interferes with the proper operation of the paper-making machine by accumulating on the screens and in the head boxes and by carrying considerable quantities of fibre, filling material and size into the waste, but also results in the formation of inferior paper having characteristic surface imperfections known as "froth spots."

The prior art rosin size emulsions, particularly those containing a large proportion of free rosin as a result of being prepared from only partially saponified wood rosin, have the further disadvantage of tending to deposit a crystalline product upon standing. This crystalline product is known in the art as "3:1 salt" and is a double salt consisting of three molecules of abietic acid and one molecule of an alkali-metal abietate. During the paper-making process it collects as a sludge in the dilution and storage tanks and constitutes a source of great inconvenience to the paper-maker.

It is accordingly an object of this invention to provide rosin size emulsions which do not induce frothing or foaming during paper-making operations. Another object is to provide rosin size emulsions which do not deposit a sludge of 3:1

salt during storage or upon dilution. Other objects will be apparent from the following detailed description of the invention.

I have found that the above objects may be attained in rosin size emulsions prepared from wood rosin which has been subjected to heat-treatment at temperatures below its decomposition temperature. Such heat-treatment should be sufficient to reduce substantially the tendency for the rosin to deposit 3:1 salt upon subsequent saponification, but should not be sufficient to destroy the crystallizability of the rosin, since heat-treatment to such an extent causes the formation of considerable amounts of rosin oils. The presence of such oils is undesirable in the size since they are not readily emulsified and are lacking in sizing value, contain corrosive constituents, and may become the cause of surface imperfections on the paper web. The size emulsions prepared according to the invention, however, contain only very small amounts of the undesirable rosin oils and at the same time are substantially free from 3:1 salt formation and foaming during paper-making operations. They are further advantageous in that they have unusual stability without the use of protective colloids, even when containing as high as 40 per cent of free rosin.

As hereinbefore mentioned, the new and improved size emulsions provided by the present invention are prepared from wood rosin which has been heat-treated to an extent sufficient to effect a substantial reduction in the tendency of its saponification product to form 3:1 salt but insufficient to destroy its crystallizability. Such heat-treatment may be carried out batch-wise simply by heating wood rosin, which has preferably but not necessarily been color-refined, for example, by selective solvent extraction, at a temperature below its decomposition temperature, e. g. between about 250° C. and about 350° C. and preferably under non-oxidizing conditions, until the desired change in the rosin has taken place.

More preferably, however, the heat-treatment is carried out continuously as described in detail in the co-pending application of Henry A. Johnstone, Serial No. 356,958, filed September 16, 1940. Such method consists essentially in passing the rosin, in molten condition and in heat-exchange relationship with the hot product, through a reaction vessel where it is subjected to a temperature between about 250° C. and about 350° C., preferably between about 280° C. and about 325° C., and under non-oxidizing conditions for

the required length of time. The reaction vessel is vented to provide exit for any gaseous or highly volatile products which may be formed, but it will be noted that the heating is carried out in such manner that substantially no distillation of the rosin takes place.

The time required to effect the desired changes in the rosin varies with the temperature at which the heat-treatment is carried out as well as with the particular type and grade of rosin employed. Ordinarily, however, it will be found that from 5 minutes treatment at 350° C. to about 5 hours treatment at 250° C. will be satisfactory. The extent of the heat-treatment may also be measured by determining the specific rotation of the rosin. Rosin which has been heat-treated until its specific rotation in the solid state has been raised from a negative value to a value above about +5° is substantially free from 3:1 salt formation, whereas rosin which has been heat-treated until its specific rotation has been raised to above +20° will have lost its crystallizability and will contain an undesirable proportion of rosin oils. Accordingly, the rosins which are suitable for use according to the invention are those whose specific rotation as determined in the solid state has been increased to a value between about +5° and +20°, preferably between about +10° and about +15°, by heating at temperatures between about 250° C. and 350° C.

The heat-treated rosin is then saponified by adding it in the solid or molten state to a hot aqueous solution of an alkali, such as sodium carbonate, potassium hydroxide, ammonia, sodium hydroxide, etc., and heating the mixture until the reaction is complete. The concentration of the aqueous alkali solution is usually so adjusted that upon completion of the reaction sufficient water is present to form a paste size of desired consistency and solids content. The proportion of alkali employed varies with the particular alkali as well as with the type of size desired. In preparing neutral sizes, for example, sufficient alkali is employed to react with all of the saponifiables in the rosin, whereas in preparing high free rosin sizes wherein the rosin is only partially saponified a smaller quantity of alkali is used, the exact proportion depending upon the proportion of free rosin desired in the size. The saponification may also be carried out in the cold, employing a variety of alkalies and special procedures adapted to modify certain characteristics of the size. For example, it may be carried out as described in U. S. Patent No. 2,134,911, whereby the size is spray-dried to form a dry finely-divided powder. Other variations will readily occur to those skilled in the art.

The dilution of the saponified heat-treated rosin to form the size emulsion may be carried out in a number of ways, the simplest of which consists merely in adding the thick size to hot water with violent agitation. The emulsion may also be formed by the so-called "gradual dilution method" which consists in thinning the size to about a 15 percent solids content with hot water and then adding the diluted size to an amount of hot water sufficient to form an emulsion of the desired strength, which is usually of about 3-5 per cent solids content, and thereafter cooling rapidly. A somewhat more efficient method of preparing the emulsion consists in heating the size and diluting it with hot water to form a 12 per cent emulsion at a tem-

perature of about 80° C. and thereafter further diluting to the desired concentration and quickly chilling by admixture with cold water. If desired, stabilizing agents, such as proteins, water-soluble gums, etc., may be incorporated into the size emulsion, although the use of such agents is not required.

The following example illustrates one way in which the principle of the invention has been applied but is not to be construed as limiting the same:

Two hundred and seventy pounds of K wood rosin was placed in a stainless steel kettle and heated at a temperature of about 300° C. for 30 minutes, after which it was cooled as quickly as possible by spraying water on the sides of the kettle. After cooling it was found that the specific rotation of the rosin in the solid state had been raised to a value of about +10.4° by the heat-treatment but that the rosin was readily crystallizable. One hundred pounds of this material was then saponified by mixing with 59 pounds of hot 22 per cent by weight aqueous sodium carbonate and heating at a temperature of about 85° C. for about 40 minutes. The rosin size so prepared was a thick paste containing about 79 per cent by weight solids, 19 per cent by weight of which was free rosin as determined by titration. This material was then emulsified to form an aqueous emulsion containing 3 per cent by weight solids by the "gradual dilution method," i. e. by diluting it with approximately 5.8 parts by weight of water at a temperature of about 80° C. and thereafter mixing the diluted size with about 3.5 parts by weight thereof of hot water with violent agitation. The emulsion so prepared was stable and did not precipitate 3:1 salt upon storage over long periods of time at elevated temperatures.

The tendency of the emulsion to form 3:1 salt was estimated quantitatively by dissolving a 50 gram sample of the heat-treated rosin from which it had been prepared in 50 grams of warm acetone, and thereafter adding sufficient dilute aqueous sodium hydroxide to neutralize one-fourth of the acids present in the rosin. The acetone solution was allowed to cool to room temperature and was seeded with a crystal of 3:1 salt. After standing for 24 hours the solution was filtered and the residue weighed, whereby there was obtained a 0.10 per cent yield of 3:1 salt. Wood rosin which had not been heat-treated yielded 29.4 per cent by weight of 3:1 salt when tested by this method.

A similar emulsion was prepared by diluting the paste size to 16 per cent concentration with distilled water at a temperature of 80° C. and thereafter further diluting to 3 per cent concentration at 90° C. The emulsion was then cooled and tested directly for 3:1 salt formation by storing in an oven maintained at 75° C. After 24 hours storage, the emulsion had acquired only a very faint turbidity, whereas similar size emulsions prepared from rosin which has not been heat-treated thicken and become completely opaque when tested in this manner.

The follow table presents data obtained by subjecting several typical rosin size emulsions prepared in a manner similar to that described above to a standard foam test under conditions simulating those encountered during paper-sizing. Comparative data are also included on similar rosin size emulsions prepared from rosin which had not been heat-treated as well as on a typical commercial size. The foaming test was

carried out by diluting 10 milliliters of the 3 per cent aqueous size emulsion with 500 milliliters of water and thereafter adding 10 per cent aqueous aluminum sulfate until the diluted emulsion had a pH of about 4.5. The mixture was then placed in a foam-testing apparatus which consists of a cylindrical glass vessel having a co-axially mounted hollow metal tube running to the bottom thereof. Within the tube is mounted a shaft carrying a propeller at its lower end. When the mixture is placed in the cylinder and the propeller rotated at high speed, air is sucked in through the hollow tube and is violently agitated with the mixture, thereby causing foaming. The height to which the foam rises in the vessel is read by means of graduations on the side of the vessel, each one-tenth inch of foam being considered as one foam unit.

Table

| Experiment No.— | Size composition      |         |            | Foam unit |
|-----------------|-----------------------|---------|------------|-----------|
|                 | Rosin                 | Solids  | Free rosin |           |
| 1.              | Heat-treated.....     | Percent | Percent    | 2         |
| 2.              | .....do.....          | 70.2    | 18.2       | 2         |
| 3.              | .....do.....          | 69.2    | 26.1       | 2         |
| 4.              | .....do.....          | 59.8    | 16.7       | 2         |
| 5.              | Not heat-treated..... | 70.0    | 19.0       | 6         |
| 6.              | .....do.....          | 71.2    | 21.8       | 6         |
|                 | Commercial size.....  | 69.8    | 20.0       | 8         |

Other modes of applying the principle of the invention may be employed instead of those explained, change being made as regards the method or ingredients employed, provided the product stated by any of the following claims, or the equivalent of such stated product, be obtained.

What we claim and desire to protect by Letters Patent is:

1. A dilute aqueous emulsion of a rosin size prepared by at least partially saponifying wood rosin which has been heat-treated at a temperature between about 250° C. and about 350° C. for

from about 5 minutes to about 5 hours, said heat-treatment being sufficient to reduce substantially the tendency of the rosin to form 3:1 salt upon subsequent saponification but insufficient to destroy its crystallizability.

2. A dilute aqueous emulsion of a rosin size prepared by at least partially saponifying wood rosin whose specific rotation in the solid state has been raised to a value between about +5° and about +20° as the result of having been heated at a temperature between about 250° C. and about 350° C. for from about 5 minutes to about 5 hours, said heat treatment being sufficient to reduce substantially the tendency of the rosin to form 3:1 salt upon subsequent saponification but insufficient to destroy its crystallizability.

3. A dilute aqueous emulsion of a rosin size prepared by at least partially saponifying wood rosin whose specific rotation in the solid state has been raised to a value between about +10° and about +15° as the result of having been heated at a temperature between about 280° C. and about 325° C. for from about 5 minutes to about 5 hours, said heat treatment being sufficient to reduce substantially the tendency of the rosin to form 3:1 salt upon subsequent saponification but insufficient to destroy its crystallizability.

4. A dilute aqueous emulsion of a rosin size prepared by at least partially saponifying wood rosin which has been heat-treated at a temperature between about 250° C. and about 350° C. for from about 5 minutes to about 5 hours to an extent sufficient to reduce substantially its tendency to form 3:1 salt upon subsequent saponification but insufficient to destroy its crystallizability, said saponification being effected by means of an aqueous alkali selected from the group consisting of sodium hydroxide and sodium carbonate.

EDMUND A. GEORGI.  
ARTHUR L. OSTERHOF.